

# UNITED STATES PATENT OFFICE.

KINGSLEY A. GILLESPIE, OF WOODBURY, NEW JERSEY, ASSIGNOR TO E. I. DU PONT DE NEMOURS & COMPANY, OF WILMINGTON, DELAWARE, A CORPORATION OF DELAWARE.

## PROCESS OF PRODUCING DESENSITIZED EXPLOSIVES AND PRODUCTS THEREOF.

1,370,015.

Specification of Letters Patent.

Patented Mar. 1, 1921.

No Drawing.

Application filed June 3, 1918. Serial No. 237,891.

To all whom it may concern:  
Be it known that I, KINGSLEY A. GILLESPIE, of Woodbury, in the county of Gloucester and in the State of New Jersey, have invented a certain new and useful Improvement in Processes of Producing Desensitized Explosives and Products Thereof, and I do hereby declare that the following is a full, clear, and exact description thereof.

10 My invention relates particularly to a process of producing desensitized explosives and the product thereof, but it has especial reference to the production of explosive compositions which are used in filling grenades.

15 The object of my invention is to provide a process by which an explosive may be desensitized, and particularly by means of which explosive compositions that are used 20 in filling grenades may be rendered insensitive, so that they will not be exploded when pierced by rifle bullets, and relates also to the product thus produced.

25 The object of my invention is, furthermore, to provide explosive compositions having the following characteristics and properties: The composition has sufficient strength to fragment the metallic envelop 30 of a grenade and drive the fragments at a high velocity to a maximum range; it is sufficiently insensitive to be pierced by a service bullet fired from a standard army rifle when contained in a cardboard container; it can be effectively detonated with 35 a blasting cap containing 1 gram of a mixture of 90 parts fulminate of mercury and 10 parts chlorate of potash; it will withstand the action of a humid atmosphere; the composition is free-running, and may be 40 readily loaded through small loading holes; and it will not begin to decompose at 65.5°C.

Still another object of my invention is to provide a process in which the explosive composition to be produced is desensitized 45 before the drying operation, which thus renders the drying operation comparatively safe.

Further objects of my invention will appear from the detailed description thereof 50 contained hereinafter.

While my invention is capable of being carried out in many different ways, for the purpose of illustration I shall describe here-

in only certain ways of carrying out the same.

For example, in carrying out my invention I may proceed as follows: A quantity of wet nitrostarch as it comes from the wringers, which may have a weight of 650.7 pounds and which may contain from 19% to 25% of water, is screened to break up the lumps, and is then mixed in a mixer of any suitable character with 6.3 pounds of an oil, as for example heavy lubricating petroleum oil, and 41.5 pounds of a solution of gum arabic carrying 12% of gum arabic and 88% of water. The gum arabic solution is of such a strength as to contain a quantity of water which, together with the water present in the nitrostarch, will give the mixture the proper consistency for graining, that is to say so as to enable the same to be formed into grains which will take the size of the mesh of the screen through which the graining is brought about. The mixture is then grained by passing through a screen having 10 meshes to the inch, and thereafter the grained mixture is dried at a temperature of from 90° to 120° F. for a period of about 40 hours.

It will thus be seen that the oil and water, which have the effect of desensitizing the mixture, are added before the drying takes place.

The oil, gum arabic and water act as desensitizing agents during drying, and the oil, gum arabic and that portion of the water which remains in the dried material desensitizes the finished explosive composition, each of said materials contributing to the desensitizing effect.

90 The dried explosive composition will then contain:

|                                 | By weight. |
|---------------------------------|------------|
| Nitrostarch                     | 97.25%     |
| Heavy lubricating petroleum oil | 1.25%      |
| Gum arabic                      | 1.00%      |
| Water                           | 0.50%      |

In the last-mentioned composition, however, considerable variation of the character and quantity of the constituents may take place, the original composition before drying being varied accordingly.

For example, the resultant composition may contain from 0.75% to 2.00% of the

oil; the gum arabic may vary from 0.75% to 2.00%; the water may range from 0.25% up to 2.00%.

Instead of the nitrostarch, furthermore, 5  
5 nitrated vegetable ivory may be used; instead of the heavy lubricating petroleum oil any other oil having a desensitizing effect may be used; and instead of the gum arabic any other water-soluble gum may 10  
10 be utilized.

While I have described my invention above in detail, I wish it to be understood that many changes may be made therein without departing from the spirit of the 15  
15 invention.

I claim:

1. The process which comprises desensitizing a composition containing a nitrated carbohydrate by providing water and an oil 20  
20 therein, at least a part of the water being present as water added in the manufacture of the explosive compound.

2. The process which comprises desensitizing a composition containing a nitrated carbohydrate by providing water and an oil therein, at least a part of the water being present as water added in the manufacture 25  
25 of the explosive compound, and then drying the same.

3. The process which comprises desensitizing a composition containing nitrostarch by providing water and an oil therein, at least a part of the water being present as water added in the manufacture of the nitro- 30  
30 starch.

4. The process which comprises desensitizing a composition containing nitrostarch by providing water and an oil therein, at 35  
35

least a part of the water being present as water added in the manufacture of the nitro- 40  
40 starch, and then drying the same.

5. An explosive containing a nitrated carbohydrate that is desensitized by the presence of water and an oil.

6. An explosive containing nitrostarch 45  
45 and a desensitizing liquid comprising an oil.

7. An explosive containing nitrostarch that is desensitized by the presence of water and an oil.

8. An explosive containing nitrostarch 50  
50 that is desensitized by the presence of a desensitizing liquid and an adhesive.

9. An explosive containing nitrostarch that is desensitized by the presence of water and an adhesive.

10. An explosive containing nitrostarch 55  
55 that is desensitized by the presence of water and an oil and an adhesive.

11. An explosive containing nitrostarch that is desensitized by the presence of a desensitizing liquid and gum arabic.

12. An explosive containing nitrostarch that is desensitized by the presence of water and gum arabic.

13. An explosive containing nitrostarch 60  
60 that is desensitized by the presence of water and an oil and gum arabic.

14. An explosive containing undried nitrostarch that is desensitized by the presence of water and an oil.

In testimony that I claim the foregoing I have hereunto set my hand.

KINGSLEY A. GILLESPIE.

Witnesses:

J. M. COWGILL,  
W. L. ARMSTRONG.